

Oct. 26, 1926.

1,604,557

P. W. JENKINS

METHOD OF MANUFACTURING DECORATIVE GLASSWARE

Filed Sept. 10, 1924



INVENTOR

Paul W. Jenkins  
By  
Winter, Brown & Critchlow  
his Attorneys.

## UNITED STATES PATENT OFFICE.

PAUL W. JENKINS, OF CHARLEROI, PENNSYLVANIA, ASSIGNOR TO MACBETH-EVANS  
GLASS COMPANY, OF PITTSBURGH, PENNSYLVANIA, A CORPORATION OF PENNSYLVANIA.

## METHOD OF MANUFACTURING DECORATIVE GLASSWARE.

Application filed September 10, 1924. Serial No. 737,009.

The invention relates to the manufacture of what is commonly known as incrusted glassware, or, more specifically described, that type of decorated glassware in which 5 the decoration consists of or includes coated relief or intaglio, both of which are herein-after referred to as relief.

The practice followed for many decades in the manufacture of decorated glassware 10 of the character herein contemplated has been first to form, usually by blowing, glass articles having plain surfaces, then to form, by the etching process, relief designs on such areas of the glass as it was desired to have 15 decorated with coated relief designs, and finally to coat the so-called relief design areas, usually with a suitable paint which is generally, but not necessarily, gold. Later 20 the coated articles are fired to set the coating. Not only does the etching step form a relief design, but it forms the design in such sharp outline, and leaves the surface in such condition that it readily retains the coating 25 subsequently applied to it.

Articles so decorated are very attractive, but they are necessarily very expensive because of the time required for, and hence 30 the expense involved in their manufacture. By far the largest item of expense is incident to the etching process for forming relief designs on the areas which are later coated. This is done by first coating an article with wax or some other material 35 which is resistant to the action of acid, then removing the wax to leave the glass exposed in a negative of the pattern which it is desired to ultimately have stand out in relief, and finally immersing the thus-prepared article in an acid which attacks the portions of 40 the surface of the glass from which the wax has been removed, and leaves the wax-covered portions stand out in relief. Later the wax is entirely removed from the article, which further adds to the expense of the 45 relief-forming step.

Aside from the expense involved in this method, it has further objectionable characteristics. When applied to thin blown glassware, and this is the type of ware to which 50 it is usually applied, the thinning of the glass by acid further weakens the inherently fragile articles. Furthermore, regardless of what type of glassware the method is applied to, the relief design cannot for prac-

tical reasons, project from or beyond the undecorated surface of an article. 55

The object of this invention is to provide a method of manufacturing decorated glassware of the type explained, whereby such glassware may be produced at a greatly reduced cost, a method which does not weaken the glassware, and a method which may be used to form relief designs which are either flush with or project beyond the undecorated 60 surfaces of glassware. 65

According to this invention the relief-forming step of the prior method of manufacture is effected simultaneously with the shaping of an article of glassware from a mass of plastic glass, it having been found 70 that a coating-retaining relief design may be so formed. A mass of plastic glass is placed in a mold having an area of its surface provided with a relief design, and pressure is applied to the mass to simultaneously shape 75 the article and to form a coating-retaining relief design on an area of its outer surface. Later an adhering coating is formed on the relief area of the article.

While the relief design may be variously 80 formed on the mold, as for example by milling or otherwise cutting the mold with tools, it is preferably formed by the etching process. In other words, the procedure which has heretofore been carried out on each 85 glass article is, according to the preferred manner of practising this invention, carried out on a mold with which thousands of articles may be manufactured. Preferably the design is etched as intaglio in the mold 90 so as to appear as a relief design on the surfaces of the articles formed in the mold. This has the advantage that the thickness 95 of the wall of the article is not diminished by the formation of the design. However, by etching or machining or both etching and machining the design may be formed as relief on the mold so as to appear as intaglio in the articles. It has been found 100 that by etching the design in the mold and by the proper application of pressure to a body of plastic glass in the mold there results the formation of a relief design on the article which is capable of retaining a coating subsequently applied to it. 105

The pressure applied to the glass to form an article with a coating-retaining relief design on its surface may be effected by

the relative approach of cooperating molds in a glass press, but is preferably effected by the blowing air used in a glass blowing machine. In either case high pressure is 5 preferably used so as to produce a relief design having a sharp outline which facilitates adherence of coating. After the article is formed, its relief design area is 10 cause the coating to adhere to the design area thus formed. As previously indicated, the coating is preferably gold, but may be silver or other colors.

In the accompanying drawing there is 15 shown a perspective view of a thin blown tumbler manufactured according to the method herein disclosed, the outer surface of its mouth being provided with a coated relief band. It has been found that decorated tumblers of the type so illustrated 20 may be manufactured according to this method at a cost less than one fifth of that incident to the method of manufacture which has been followed for decades; that 25 tumblers manufactured according to this method have the same appearance as those made according to the old method; and that the coating adheres to the relief area

just as firmly as if the relief area of each article were formed on the article by the 30 etching process.

I claim:

1. The method of manufacturing an in-crusted glass article, which comprises blowing a mass of plastic glass within a mold having an area of its surface provided with a relief design, and by such blowing simultaneously shaping the article and forming a shallow coating-retaining relief design of sharp outline on an area of the outer surface of the article, and subsequently forming an adherent coating on said relief area of the article. 40

2. The method of manufacturing an in-crusted glass article, which comprises blowing under high pressure a mass of plastic glass within a mold having an area of its surface provided with an etched relief design, and by such blowing simultaneously shaping the article and forming a shallow 45 coating-retaining relief design of sharp outline on an area of the outer surface of the article, and subsequently forming an adherent coating on said relief area of the article. 50

In testimony whereof, I sign my name.  
PAUL W. JENKINS